

## UNITED STATES PATENT OFFICE

2,286,870

## MAGNESIUM BASE ALLOY

John C. McDonald, Midland, Mich., assignor to  
The Dow Chemical Company, Midland, Mich.,  
a corporation of Michigan

No Drawing. Application December 23, 1940,  
Serial No. 371,379

2 Claims. (Cl. 75—168)

The invention relates to magnesium base alloys and more particularly concerns an alloy of this nature having a high degree of formability associated with other desirable physical properties, such as excellent tensile and yield strengths.

Magnesium base alloys are being widely used in the structural arts where a lightweight metal is highly desirable, such as for use in making castings, forgings, and the like. However, the use of these alloys in the rolled form to make sheet metal articles requiring forming operations, such as bending and drawing, has not progressed as rapidly due to the fact that, in general, alloys having good formability or ductility permitting relatively sharp bends to be made without the article developing external cracks, usually have inferior characteristics as regards their tensile and yield strengths.

It is, accordingly, the principal object of the invention to provide a magnesium base alloy which can be made into rolled sheet and the like possessing a sufficient degree of ductility or formability at ordinary temperatures to be sharply bent, drawn or otherwise shaped, while having good tensile and yield strengths.

Other objects and advantages will be apparent as the description of the invention proceeds.

My invention resides in the discovery that a magnesium base alloy containing from 0.01 to 1 per cent of calcium, from 0.01 to 1 per cent of cerium, and from 1 to 15 per cent of thallium possesses the aforementioned desirable properties. The term "magnesium" used herein and in the appended claims is intended to include magnesium containing the ordinary impurities that are found in the commercially pure metal, such as traces of iron, copper, nickel, and silicon. While the properties of improved ductility or formability associated with high tensile and yield strengths are manifest over the entire range of composition indicated, a particularly desirable composition, because of its combination of properties is one containing 0.2 per cent calcium, 0.2 per cent of cerium, and 5 per cent of thallium.

The following table, listing some of the properties of rolled sheet made from my new alloy and comparing these properties with those of some related alloys, illustrates the improvement in formability, yield and tensile strengths shown by the new alloy.

In the table, the per cent elongation is to be regarded as a measure of the ductility or formability of the alloys.

Table

| 5  | Nominal composition in percent (magnesium=remainder) |     |    | Annealed                        |                                |                                  |
|----|------------------------------------------------------|-----|----|---------------------------------|--------------------------------|----------------------------------|
|    | Ce                                                   | Ca  | Tl | Per cent elongation in 2 inches | Yield strength in lbs./sq. in. | Tensile strength in lbs./sq. in. |
| 10 | ...                                                  | 0.3 | 5  | 15                              | 21,000                         | 35,000                           |
| 15 | 0.2                                                  | 0.2 | —  | 18                              | 20,000                         | 34,000                           |
| 20 | 0.2                                                  | 0.2 | 5  | 19                              | 23,000                         | 35,000                           |

The properties set forth above under the term "annealed" were obtained by first rolling the alloys at a temperature of 550° F. and thereafter annealing them at various temperatures through a range of from 400 to 800° F. The properties selected for the table were those of the annealed specimens which exhibited the maximum elongation.

A comparison of the properties listed in the above table shows that the new alloy possesses superior formability characteristics coupled with improved yield and tensile strengths. The improvement noted in the composition listed is exhibited throughout the percentage range of alloying ingredients indicated.

While the new alloy is most useful in wrought form, such as sheets, due to its formability characteristics, it may also be used for making castings, extruded forms, and the like.

The new alloy may be compounded by any of the methods usually employed for melting and alloying metals with magnesium such as by adding the alloying ingredient singly or jointly to a bath of molten magnesium which is preferably protected from oxidation by suitable flux. The flux should be substantially free from magnesium chloride, if the calcium content of the alloy is above 0.3 per cent. In those instances where the alloy is to be compounded containing less than 0.3 per cent of calcium, magnesium chloride may be present in the flux, but in this case it is preferable to add the calcium last without too much stirring or agitation in order to prevent loss of calcium into the flux. Cerium may be added to the alloy as such, or in the form of Misch-metal. Magnesium-cerium alloys are commonly made up by employing Misch-metal as a source of cerium. It is sometimes desirable to add more than the theoretical amount of Misch-metal since the alloying efficiency is not always 100 per cent and some loss may be incurred.

It is to be understood that the invention is not limited to the specific composition herein described, but may take other forms without departing from the scope of the invention.

I claim:

1. A magnesium base alloy containing 0.01 to 1 per cent of calcium, from 0.01 to 1 per cent

of cerium, and from 1 to 15 per cent of thallium, the balance being magnesium.

2. A magnesium base alloy containing 0.2 per cent of calcium, 0.2 per cent of cerium, and 5 per cent of thallium, the balance being magnesium.

JOHN C. McDONALD.